

## FREE FLOWING CYCLOTRIMETHYLENE-TRINITRAMINE

William Earle Schulz, Wenonah, N. J., assignor to E. I. du Pont de Nemours and Company, Wilmington, Del., a corporation of Delaware

No Drawing. Application March 23, 1953,  
Serial No. 344,194

3 Claims. (Cl. 260—248)

The present invention relates to a method for improving the flowing properties of cyclotrimethylenetrinitramine.

Cyclotrimethylenetrinitramine can be recovered from compositions in which it was mixed with trinitrotoluene, dinitrotoluene, mononitrotoluene, tetryl, and nitrocotton in the form of finely divided particles which pass a 50 mesh screen. This finely divided cyclotrimethylenetrinitramine is not suitable for direct use in new explosive compositions because of its poor flowing properties which make handling difficult. Cyclotrimethylenetrinitramine of suitable particle size can be obtained by recrystallization from a suitable solvent, but this method of improving flowing properties involves considerable expense. Moreover, the suitable solvents are highly flammable and introduce a fire hazard which is particularly undesirable where explosives are involved.

Mechanical mixing of calcium stearate with finely divided explosive compounds is frequently used to produce compositions with improved flowing properties. The calcium stearate has the added advantage of acting as a desensitizer and a mold lubricant for most explosive compounds. However, when mixed with finely divided cyclotrimethylenetrinitramine, calcium stearate produces a flocculent solid having only fair flowing properties.

An object of the present invention is to provide a process for improving the flowing properties of finely divided cyclotrimethylenetrinitramine. Another object of the present invention is to produce free-flowing cyclotrimethylenetrinitramine as a result of combination with a water-insoluble metallic salt of a high molecular weight fatty acid. A still further object of this invention is to provide a process for the uniform intermingling of calcium stearate or a similar water-insoluble metallic salt of a high molecular weight fatty acid with finely divided cyclotrimethylenetrinitramine, even when fractional percentages of the salt are to be used with the explosive compound. Additional objects will become apparent as the invention is further described.

I have found that the foregoing objects may be accomplished by treating the cyclotrimethylenetrinitramine dispersed in a water slurry with a water-soluble salt of high molecular weight fatty acid, and thereafter adding to said water slurry a water-soluble salt of a metal which forms a water-insoluble metallic salt of said fatty acid.

In accordance with the process of this invention, finely divided, water-insoluble cyclotrimethylenetrinitramine is suspended in water with vigorous agitation and 0.5-5% by weight of a water-soluble salt of a solid fatty acid having more than 10 carbon atoms is added. To this aqueous slurry is added an excess of an aqueous solution of a salt of a metal capable of forming a water-insoluble salt with the fatty acid. Typical salts of this type are calcium chloride, magnesium chloride, zinc chloride, lead chloride, and nickel chloride. The insoluble precipitate thus formed coats the larger grains of cyclotrimethylenetrinitramine and agglomerates the finer crystals during the precipitation.

The dustiness usually produced when solid, water-insoluble metallic salts of fatty acids are mixed mechanically with crystalline compounds is thus avoided by the present method of forming the insoluble coating by precipitation from an aqueous solution in the presence of the explosive compound. Moreover, various amounts of the agent may be added and a more intimate mixture obtained.

Ordinary hand soap and alkali metal salts of stearic acid may be used as the source of the water-soluble coating agent. Solid fatty acids having more than 10 carbon atoms, especially those with an even number of carbon atoms, are preferred, and the fatty acids are added in amounts of 0.5-5% by weight of the explosive compound.

Water-soluble salts of metals such as calcium, magnesium, zinc, and nickel may be used to precipitate the fatty acid, calcium chloride being the preferred salt. The amount required will depend upon the quantity of fatty acid in the aqueous mixture, and preferably an excess of the water-soluble precipitating salt will be added. The following examples illustrate specific embodiments of the method of carrying out the present invention. It should be understood, however, that they are illustrative only and are not to be taken as limiting the invention.

*Example 1*

To a slurry of 500 parts of cyclotrimethylenetrinitramine and 500 parts of warm water containing 15 parts (3% by weight) of dissolved soap, i. e. sodium stearate, was added, slowly, with constant agitation, 12 parts of calcium chloride in 100 parts of water. The solid obtained was filtered and dried. The treated cyclotrimethylenetrinitramine had excellent flowing properties.

*Example 2*

Two hundred parts of finely divided cyclotrimethylenetrinitramine was mixed with 0.5% of a fatty alcohol sulfate in 500 parts of water. The fatty alcohol sulfate was added to reduce any static electricity on the cyclotrimethylenetrinitramine. Ten parts of soap, i. e. sodium stearate (5% by weight), was added and the slurry heated to 45° C. A solution of 5 parts of calcium chloride in 100 parts of water was slowly added to the well-agitated slurry. The solid obtained was filtered and dried. The treated cyclotrimethylenetrinitramine had excellent flowing properties.

Although the invention has been described in detail in the foregoing description, it will be apparent that many variations may be made without departing from the basic inventive concept. It is intended, therefore, to be limited only in accordance with the following claims:

I claim:

1. A process for producing cyclotrimethylenetrinitramine with improved flowing properties comprising forming a slurry of cyclotrimethylenetrinitramine particles in warm water, adding thereto from 0.5-5% by weight of a water-soluble salt of a fatty acid and thereafter adding to said slurry an excess of an aqueous solution of a water-soluble salt of a metal which forms an insoluble salt with said fatty acid.

2. A process for producing cyclotrimethylenetrinitramine with improved flowing properties comprising forming a slurry of the cyclotrimethylenetrinitramine in warm water, adding to said slurry 0.5-5% by weight of a solution of potassium stearate, and thereafter adding to said slurry an excess of an aqueous solution of calcium chloride.

3. A process for producing cyclotrimethylenetrinitramine with improved flowing properties, comprising forming a slurry of said cyclotrimethylenetrinitramine in warm water; adding thereto 0.5-5% by weight of a soluble salt

of a normally solid fatty acid of over 10 carbon atoms; agitating the slurry; and thereafter adding to the slurry, with mixing, an aqueous solution of a salt of a metal selected from the group consisting of calcium, magnesium, zinc, lead and nickel.

|         |       |               |
|---------|-------|---------------|
| Nichol  | ----- | Mar. 8, 1932  |
| Baldwin | ----- | Feb. 6, 1934  |
| Meister | ----- | Apr. 5, 1938  |
| Lewis   | ----- | July 19, 1938 |

## FOREIGN PATENTS

|               |       |               |
|---------------|-------|---------------|
| Great Britain | ----- | Dec. 31, 1945 |
| Great Britain | ----- | 1946          |

## References Cited in the file of this patent

## UNITED STATES PATENTS

|           |      |                |    |
|-----------|------|----------------|----|
| 1,728,307 | Ripp | Sept. 17, 1929 | 10 |
|-----------|------|----------------|----|

|         |
|---------|
| 574,271 |
| 579,302 |